

## UNITED STATES PATENT OFFICE

CAMILLE DREYFUS, OF NEW YORK, N. Y.

## PLAITED FABRIC AND PROCESS OF PRODUCING THE SAME

No Drawing.

Application filed July 15, 1927. Serial No. 206,119.

This invention relates to a process of plaiting woven, knitted or other fabrics made of or containing thermoplastic derivatives of cellulose. The term thermoplastic derivatives of cellulose is to be interpreted as including the various esters and ethers of cellulose which are rendered plastic by heat. Cellulose nitrate, cellulose acetate, cellulose butyrate, methyl cellulose, ethyl cellulose, etc., 5 may be cited as examples of such thermoplastic derivatives. While such fabrics have been plaited heretofore the results obtained were not permanent in nature and disappeared upon being dampened or upon continued wear, particularly in damp atmospheres. In this respect the plaiting of fabrics containing thermoplastic derivatives of cellulose gave results very similar to those obtained when plaiting fabrics of other 15 textile materials.

An object of this invention is to provide a process whereby the plaitings of fabrics containing thermoplastic derivatives of cellulose can be very effectively accomplished. Another object of this invention is to produce plaitings on fabrics containing thermoplastic derivatives of cellulose which shall be permanent—or at least much more permanent than heretofore. Another object of this invention is to devise a process for producing plaitings on fabrics containing organic derivatives of cellulose which will not be removed when the fabric is subjected to laundering operations. Other objects and advantages of this invention will appear from the description and claims.

The usual process of plaiting consists in passing the fabric together with a paper between rolls so adjusted and faced as to give 40 plaita of the desired size and configuration. In some instances best results are obtained by protecting the fabric, above and below, with paper while the same passes between the rolls of the plaiting machine. As previously stated, however, the plaitings thus obtained are not permanent.

The present invention consists in my discovery that the plaiting of woven or knitted fabrics made of or containing thermoplastic derivatives of cellulose can be made permanent.

55

agent if the fabric is treated with a softening agent prior to subjecting it to the plaiting operation. The plaiting thus obtained is permanent, persisting even when the fabric is subjected to laundering operations

55

One method of carrying out my invention will now be described. A fabric containing cellulose acetate yarns which was to be plaited in accordance with my invention was sprayed with a dilute (25%) aqueous solution of acetone. The excess liquid was then removed by passing the fabric through nip rolls. The slightly damp fabric was then passed through a Chandler plaiting machine under the usual conditions, except that the apparatus may be maintained at a lower temperature than usual. The fabric was found to have been beautifully and permanently plaited. Its snap or spring-back was much superior to that usually obtained upon plaiting ordinary fabrics in the usual way. In addition to the improved snap or spring-back it was found that the fabric had not been delustered or at all discolored by the steaming to which it had been subjected in the plaiting operation. This is a material advantage since natural silk and other fabrics turn yellow as a result of the steaming which they receive in the plaiting process.

70

75

80

85

90

95

My invention is not to be considered as limited to the above specific embodiment. Fabrics containing thermoplastic derivatives of cellulose other than cellulose acetate were treated as outlined above and similar beneficial results were obtained. The concentration of the dilute aqueous acetone can also be varied and where desired can be replaced by dilute solutions of other solvents or by solutions of softening agents for the particular thermoplastic derivative of cellulose present in the fabric. Where solvents of the thermoplastic derivative of cellulose are employed they should be so diluted that they will not destroy or otherwise deleteriously affect the fabric; where solid softening agents are employed they should be dissolved in a solvent which will not deleteriously affect the fabric being treated.

100

Instead of spraying the solution of the solvent or the softening agent of the thermo-

plastic derivative of cellulose onto the fabric the latter can be dipped in or otherwise impregnated with the solvent or softening agent. The excess liquid can be removed 5 from the fabric by evaporation or whizzing as well as by passing the fabric between nip rollers.

The process above outlined can be modified by wetting or impregnating the protecting

10 paper utilized in the process with the solvent or softening agent for the thermoplastic derivative of cellulose instead of similarly wetting the fabric itself. In this modification when upper layers and lower layers of paper 15 are employed it is necessary to thus wet only one of the protecting layers of paper. (The paper thus wetted should have a capacity for retaining a certain proportion of the softening agent solution applied thereto.)

20 The amount of softening agent or solvent employed in this process can be varied as desired even to the point of dispensing with its use altogether. The smaller the amount of softening agent employed the higher will be 25 the temperature and pressure necessary to effect the permanent plaiting of the fabric containing the thermoplastic cellulose derivative. Thus where no softening agent is employed the temperature and pressure will 30 have to be raised to the point where the cellulose derivative becomes plastic in order to obtain a permanently plaited fabric. Usually it is advantageous to employ at least a slight amount of softening agent.

35 The term "softening agent" as used in the description and claims includes within its scope any compounds which have a swelling, softening or solvent action upon the thermoplastic derivative of cellulose present in the 40 fabric. It also embraces the use of such compounds alone or when used in conjunction with solvents or diluents which may or may not affect the thermoplastic derivative of cellulose at the temperature at which the plaiting is carried out.

45 As examples of solvents for cellulose acetate the following are mentioned: acetone, diacetone alcohol, cyclohexanone, alcohol, aceto-acetic ester, acetic acid, ethyl lactate, 50 etc., and as examples of swelling agents, solutions of ammonium thiocyanate, stannic chloride, etc., may be given. Non-volatile softening agents such as triacetin, triphenyl phosphate, sulfonamides of aromatic compounds such as mono methyl ethylene sulfonamide, p-toluene sulfonamide, etc., may also 55 be employed. The wetting liquid may also contain a lubricant such as oleic acid, ammonium oleate, olive oil etc., for the purpose of 60 reducing the internal friction in the fabric.

65 The improved results obtained by treating fabrics containing cellulose acetate with dilute aqueous acetone were duplicated when other thermoplastic derivatives of cellulose 70 and other solvents or softening agents were

employed. My invention is not dependent upon the use of a Chandler type of plaiting machine as other types of plaiting machines were successfully substituted in carrying out my process. My invention, therefore, is not 75 to be construed as limited to the specific illustration previously given but is to be considered as limited only by the scope of the appended claims.

Having described my invention what I 75 claim and desire to secure by Letters Patent is:

1. A process of plaiting a fabric containing 80 yarns of thermoplastic derivatives of cellulose which comprises subjecting the fabric to a suitable plaiting operation at a temperature and pressure sufficiently high to render the cellulose derivative plastic, whereby the fabric is permanently plaited.

2. A process of plaiting a fabric containing 85 yarns of organic derivatives of cellulose which comprises subjecting the fabric to a suitable plaiting operation at a temperature and pressure and pressure sufficiently high to render the cellulose derivative plastic, whereby the 90 fabric is permanently plaited.

3. A process of plaiting a fabric containing 95 yarns of cellulose acetate which comprises subjecting the fabric to a suitable plaiting operation at a temperature and pressure sufficiently high to render the cellulose acetate plastic, whereby the fabric is permanently 100 plaited.

4. A process of plaiting a fabric containing 105 yarns of thermoplastic derivatives of cellulose which comprises subjecting the fabric to a suitable plaiting operation in the presence of a softening agent for the thermoplastic derivative of cellulose, whereby the fabric is permanently plaited.

5. A process of plaiting a fabric containing 110 yarns of cellulose acetate which comprises subjecting the fabric to a suitable plaiting operation in the presence of a softening agent for the cellulose acetate, whereby the fabric is permanently plaited.

6. A process of permanently plaiting fabrics containing yarns of thermoplastic derivatives of cellulose which comprises treating the fabric with a softening agent for the thermoplastic derivative of cellulose and then subjecting the fabric to any suitable plaiting operation.

7. A process of permanently plaiting fabrics containing yarns of thermoplastic derivatives of cellulose which comprises treating the fabric with an aqueous solution of a softening agent for the thermoplastic derivative of cellulose and then subjecting the fabric to any suitable plaiting operation.

8. A process of permanently plaiting fabrics containing yarns of thermoplastic derivatives of cellulose which comprises treating the fabric with an aqueous solution of

acetone, and then subjecting the fabric to any suitable plaiting operation.

9. A process of permanently plaiting fabrics containing yarns of thermoplastic derivatives of cellulose which comprises treating the fabric with a 25% aqueous solution of acetone, and then subjecting the fabric to any suitable plaiting operation.

10. A process of permanently plaiting fabrics containing yarns of thermoplastic derivatives of cellulose which comprises treating the fabric with an aqueous solution of acetone, removing the excess liquid and then subjecting the fabric to any suitable plaiting operation.

11. A process of permanently plaiting fabrics containing yarns of cellulose acetate which comprises treating the fabric with a softening agent for the cellulose acetate and then subjecting the fabric to any suitable plaiting operation.

12. A process of permanently plaiting fabrics containing yarns of cellulose acetate which comprises treating the fabric with an aqueous solution of acetone, and then subjecting the fabric to any suitable plaiting operation.

13. A process of permanently plaiting fabrics containing yarns of cellulose acetate which comprises treating the fabric with a 25% aqueous solution of acetone, and then subjecting the fabric to any suitable plaiting operation.

14. A process of permanently plaiting fabrics containing yarns of cellulose acetate which comprises treating the fabric with an aqueous solution of acetone, removing the excess liquid and then subjecting the fabric to any suitable plaiting operation.

15. A fabric containing yarns of a thermoplastic derivative of cellulose which possesses plaits which are permanent in nature.

16. A fabric containing yarns of a fatty acid ester of cellulose which possesses plaits which are permanent in nature.

17. A fabric containing yarns of cellulose acetate and a softening agent therefor which possesses plaits which are permanent in nature.

50 In testimony whereof, he has hereunto subscribed his name.

CAMILLE DREYFUS.